

Patented Jan. 29, 1929.

1,700,596

# UNITED STATES PATENT OFFICE.

GEORGE A. RICHTER, OF BERLIN, NEW HAMPSHIRE, ASSIGNOR TO BROWN COMPANY, OF BERLIN, NEW HAMPSHIRE, A CORPORATION OF MAINE.

## COMPOSITION FOR CONVERSION INTO CELLULOSE DERIVATIVES AND PROCESS OF PREPARING SAME.

No Drawing.

Application filed March 3, 1927. Serial No. 172,568.

In my application, Serial No. 77,624, filed December 24, 1925, there is disclosed and claimed a process of producing high alpha cellulose wood fiber particularly adapted for the preparation of cellulose derivatives such as cellulose xanthate. In accordance with that process, a raw or unbleached pulp, pre-treated if desired with an oxidizing or chlorinating reagent, is treated with caustic soda solution of mercerizing strength to effect a solution and removal of non-alpha cellulose constituent therefrom and accordingly a refinement of such pulp to a high alpha cellulose content. Such pulp, when bleached, constitutes an excellent material for the preparation of cellulose derivatives such as xanthate and nitrocellulose. Also, in application, Serial No. 140,677, filed October 9, 1926, the advantages of mercerizing wood pulp, but more particularly a bleached high alpha cellulose wood pulp, prior to conversion into such derivatives as the nitrocellulose, are disclosed. In such latter case, mercerization of the pulp in bulk form, particularly in the presence of a small quantity of an oxidant, results in a product which when nitrated and dissolved in a suitable solvent yields solutions of lower viscosity and of markedly better color than those prepared from nitrated, unmercerized pulp.

The present invention has for its object to decrease the acid retention and increase the nitrocellulose yield when pulp is mercerized in bulk form rather than in thin paper or tissue form, and then nitrated, as upon nitration the acid retention of such bulk pulp is appreciably higher and the yield appreciably lower than when unmercerized pulp is made into tissue which is mercerized and then nitrated as described in application, Serial No. 140,675, filed October 9, 1926, by Milton O. Schur and Royal H. Rasch. The quality of the nitrocellulose obtained from mercerized bulk pulp and the physical and chemical characteristics of films, lacquers, or other products prepared from such nitrocellulose are apparently as good as when similar pulp in tissue form is nitrated. The higher acid retention and lower yield are believed to be attributable to the higher absorptivity of mercerized fiber in bulk form over that in paper form. Thus, owing to the higher retention of acid by the bulk fiber, a greater loss of the fiber apparently takes place during nitration and when after centrifuging it is submerged in water,—my theory being that the wash water effects a slower dilution and washing out of the acid in the bulk fiber than when tissue is washed, and that during such slower dilution, acid concentrations are produced in the bulk fiber which favor a hydrolysis of nitrocellulose.

If, however, it be attempted to form paper or tissue from the mercerized fiber prior to nitration, difficulty is experienced, as mercerized fiber is unhydratable, and even after long beating, if such beaten fiber is run off on a papermaking machine, a loose, bulky paper of non-uniform thickness results, which upon nitration yields practically no improvement over bulk pulp. Even if the mercerized pulp be beaten many times as long as is usually necessary for unmercerized pulp, the paper formed therefrom is altogether too loose and bulky to improve nitration results.

I have found that if mercerized pulp, and more particularly mercerized alpha pulp, is uniformly mixed with unmercerized beaten or unbeaten pulp, the composite pulp may be formed into a tissue or light weight paper which yields materially improved results upon nitration. For instance, the mercerized pulp may be uniformly mixed with a relatively small proportion of well-beaten, unmercerized pulp, as in a hollander. Or the mercerized pulp may be uniformly mixed with unbeaten, unmercerized pulp and then beaten until sufficient hydration of the unmercerized pulp has been effected to bond the mercerized pulp together into a well-felted tissue. Preferably, however, the first-mentioned procedure of uniformly mixing a well-beaten pulp with the mercerized pulp is practised, in order to conserve power and to preserve the length of mercerized fiber, as beating merely macerates or shortens such fiber without effecting any appreciable hydration thereof. Tissue thus formed, when nitrated, has a notably lower acid retention and gives an appreciably higher nitrocellulose yield than mercerized pulp in bulk form. Preferably, such tissue is calendered in the course of its manufacture, as calendering compacts it and further enhances its suitability for nitration.

In producing tissue such as herein desired, the following mode of procedure has been found to give proper results. Sulphite fiber,

alpha fiber, cotton fiber, or the like, is treated in shredded or bulk condition with a caustic soda solution of mercerizing strength. The treatment may, for instance, be carried out 5 by the treating process and in the apparatus disclosed and claimed in my application, Serial No. 128,398, filed August 10, 1926, for example. A small quantity of an oxidant, such as sodium hypochlorite, may be added 10 to the solution, particularly when an unbleached or partially bleached fiber is being mercerized, as the oxidant reacts with and removes coloring matter from the pulp. Sulphite fiber is preferably mercerized in an unbleached or only partially bleached condition, as described in my application, Serial No. 77,624, filed Dec. 24, 1925, for if bleached sulphite pulp is mercerized, an appreciable loss and degradation of its alpha cellulose content 15 takes place. The mercerized sulphite fiber may then be bleached to the desired whiteness. After mercerization, about 5% of an over-beaten high alpha cellulose-containing fiber is uniformly disseminated throughout 20 the mercerized fiber, as by circulation or beating for a while in a hollander or other beater. Or 5% to 10% of unbeaten, unmercerized fiber may be added to the mercerized fiber, and the mixture then beaten until the desired 25 hydration of the unmercerized fiber has been effected. The composite fiber is run off on a paper machine into thin paper or tissue suitable for nitration. Such tissue is well-felted and relatively dense, so that nitration results 30 in appreciable improvement in both acid retention and yield.

The composition of mercerized, and beaten, unmercerized fiber may be produced from the same fiber or from different fiber. For instance, the mercerized fiber may be mercerized sulphite fiber, and unmercerized, beaten fiber may be alpha wood fiber or cotton fiber, alone or in admixture; or both the mercerized fiber and beaten, unmercerized fiber may be 45 produced from a high grade sulphite fiber. While for best results the composition is made into tissue, nevertheless such a composition of mercerized fiber and beaten, unmercerized fiber, when nitrated in bulk form, gives 50 improved results over a composition of mercerized fiber alone. Thus, the composition of the present invention may be fluffed mechanically to resemble cotton linters, or may be formed on a cylinder machine or Fourdrinier 55 wire from a very dilute suspension of pulp into a relatively thick, porous sheet, and dried on the mold or wire, either with or without squeezing, and nitrated in such form.

The great utility of the process herein described is that the advantages of mercerizing fiber in bulk form prior to nitration, as well as the advantages arising from a desirable physical condition of fiber when nitration is being effected, are both realized. In plant

practice, it is more economical to mercerize and wash pulp in large quantities in bulk form and to recover the mercerizing solution, rather than to mercerize a sheet or tissue. By the process of the present invention, economical advantages of mercerizing fiber in bulk form are enjoyed, and at the same time a tissue of good nitrating characteristics may be manufactured therefrom.

Having thus described my invention, it is obvious that it is subject to change and modification without departing from its spirit or scope as set forth in the appended claims.

What I claim is:

1. A cellulose fiber composition comprising a mixture of mercerized and unmercerized fiber. 80

2. A cellulose fiber composition comprising a mixture of mercerized fiber and beaten, unmercerized fiber.

3. A cellulose fiber composition comprising a substantially homogeneous mixture of a preponderant proportion of mercerized fiber and a subordinate proportion of beaten, unmercerized fiber. 85

4. A paper comprising mercerized and unmercerized cellulose fiber. 90

5. A paper comprising mercerized cellulose fiber uniformly interfelted with beaten, unmercerized cellulose fiber.

6. A process step which comprises running off on a paper machine a mixture of mercerized and unmercerized cellulose fiber. 95

7. A process which comprises running off on a paper machine a substantially uniform mixture of mercerized and unmercerized cellulose fiber and calendering the paper. 100

8. A process which comprises uniformly mixing mercerized and unmercerized cellulose fiber, and running the mixture off on a paper machine. 105

9. A process which comprises uniformly mixing mercerized cellulose fiber and unmercerized, beaten cellulose fiber, and running the mixture off on a paper machine.

10. A process which comprises running off on a paper machine a mixture of mercerized and unmercerized cellulose fiber, and converting the resulting paper into a cellulose derivative. 110

11. A process which comprises running off on a paper machine a substantially uniform mixture of mercerized cellulose fiber and beaten, unmercerized cellulose fiber, and nitrating the resulting paper. 115

12. A process which comprises uniformly mixing mercerized cellulose fiber and unmercerized, beaten cellulose fiber, running the mixture off on a paper machine, and nitrating the resulting paper. 120

In testimony whereof I have affixed my signature.

GEORGE A. RICHTER.